

# UNITED STATES PATENT OFFICE.

ERNEST WYNDHAM MERRY, OF SHEFFIELD, ENGLAND, ASSIGNOR TO PYROTAN LEATHER CORPORATION, OF WILMINGTON, DELAWARE, A CORPORATION OF DELAWARE.

## TANNING HIDES AND SKINS.

1,415,671.

Specification of Letters Patent. Patented May 9, 1922.

No Drawing.

Application filed February 11, 1919. Serial No. 276,841.

To all whom it may concern:

Be it known that I, ERNEST WYNDHAM MERRY, a subject of Great Britain, residing at Sheffield, in the county of York, England, 5 have invented certain new and useful Improvements in Tanning Hides and Skins; and I do hereby declare the following to be a full, clear, and exact description of the invention, such as will enable others skilled 10 in the art to which it appertains to make and use the same.

This invention relates to the tanning of hides and skins, and more particularly to a process wherein the advantages of chrome 15 tanning are combined with those incident to the use of a mixture of soluble pyrophosphate and alum as the principal tanning agents.

The object of my invention therefore is 20 to produce a desirable and highly satisfactory leather at a relatively slight cost which is resistant to heat and moisture and is adaptable to a wide variety of purposes.

The use of a soluble pyrophosphate in 25 connection with alum and salt has been described in Letters Patent #1,039,150 and #1,191,527. According to the process described therein, the hides are subjected after the usual preliminary cleansing and unhairing treatment, to solutions comprising alum, 30 common salt, and sodium pyrophosphate under specified conditions, to convert the hide into a superior quality of leather. For certain purposes it is desirable that the 35 leather exhibit an extreme resistance to heat and moisture and I have discovered that a leather adapted to such special purposes may be economically manufactured through the combination of pyrophosphate tanning 40 and chrome tanning as hereinafter described.

It is possible to accomplish this desirable 45 result, either by subjecting the hides to a combined solution containing the essential ingredients to accomplish both the pyrophosphate and chrome tanning, or by first subjecting the hides to a pyrophosphate tanning and subsequently treating them with a chrome tanning liquor, whereby the desirable 50 features of chrome tanning are imparted to the resulting leather.

In carrying out my invention, the hides or skins are preferably subjected to the usual washing, liming, unhairing, and fleshing op-

erations, after which they may be bated and 55 finally washed in water or suitable cleansing solutions until thoroughly clean and in suitable condition for the actual tanning operations. The details of the preliminary treatment form no part of my present invention, and may be widely varied in accordance with established practice in tan- 60 yards or otherwise.

The prepared hides are then subjected in a 65 suitable receptacle for example, a pit, drum, wheel, or paddle, to the action of a tanning solution which includes a suitable proportion of a soluble pyrophosphate, a soluble aluminum salt, and a suitable material such as sodium chloride or common salt, for over- 70 coming the astringent action of the aluminum salt upon the hide, whereby it is maintained in a porous condition to assimilate the active tanning agents. Preferably, sodium pyrophosphate, ammonia alum, and 75 common salt are employed although other soluble pyrophosphates may be substituted and any soluble aluminum salt may be advantageously used. For example, soda alum, potash alum, aluminum sulphate, or 80 aluminum chloride may be substituted for the ammonia alum.

According to one modification of the process I subject the hides to the action of the chrome liquor simultaneously with the pyrophosphate and preferably add the chrome liquor gradually to the solution in the receptacle during the tanning operation. The chrome liquor employed may be any of the usual liquors readily obtainable in the 85 market and commonly employed in chrome tanning. Such a liquor for example, may include chrome alum which has been rendered basic by the addition of a suitable alkali such as sodium carbonate, but it is to 90 be understood that my invention contemplates the employment of any of the usual and well known single bath chrome tanning agents of which there are a number available. The proportions of the various ingredients of the tanning solution, and particularly the proportion of the chrome liquor to the pyrophosphate mixture will depend entirely upon the particular purpose to be 95 accomplished, as well as upon the character 100 of the material under treatment. The hide after remaining in the combined tanning solution during a sufficient time interval to 105

accomplish thorough tanning, is withdrawn and treated in accordance with the usual practice to produce finished leather.

According to another modification of my invention, the hide is first subjected under suitable conditions to a tanning solution consisting of a soluble pyrophosphate, soluble aluminum salt, and common salt, in a suitable receptacle as above described, until the tanning of the hide is practically completed. The chrome liquor is then added directly to the spent solution in the receptacle and remains in contact with the hide for a sufficient period to impart the desired qualities thereto.

The concentration of the solution employed, with reference to the several salts contained therein, may vary somewhat depending upon the particular character of the hide treated. Preferably the proportion of pyrophosphate to the alum is maintained at a relatively low ratio which may, however, vary from 1:4 to 1:10. The higher proportions of pyrophosphate are desirable where the hides are heavy and of close texture, and the lower proportions are desirable in the treatment of hides and skins of relatively light weight and loose texture. For general purposes the range of relative proportions of alum to pyrophosphate may be limited so that the alum exceeds 5 but does not exceed 7 times the weight of pyrophosphate. The proportion of standard chrome liquor will vary from a fraction of one per cent upward to eight per cent of the weight of the hide substance, but the higher percentages will rarely be necessary inasmuch as the entire purpose of the chrome liquor is to impart certain desirable qualities to the leather which has been already tanned by the pyrophosphate solution.

The process, whether practiced by the gradual addition of the chrome liquor to the pyrophosphate solution, or by the addition of the chrome liquor after completion of the pyrophosphate tannage, results in a product having the desirable characteristics imparted by both methods of tanning and is completed at a relatively low cost, as compared with the ordinary application of chrome tannage. The product for example will be substantially moisture-proof and heat-resistant and may be subjected therefore to certain manufacturing operations, whereby a more delicate leather would be injured through the application of heat or moisture

to the finished product. Moisture proof and heat resistant leathers have moreover, many applications in the arts, which the product of the process herein described is well adapted to meet.

In the foregoing it will be readily understood that I have perfected an improved process of treating hides and skins whereby certain desirable results are accomplished and that variations may be made in the process, as well as in the ingredients employed, without departing from the invention or sacrificing any of the material advantages thereof.

I claim:

1. A method of combined tannage of hides and skins, to produce heat and moisture resistant leather, which comprises subjecting the hide to the tanning action of a solution including a soluble pyrophosphate and a soluble aluminum salt in relative proportions varying from 1:4 to 1:10, and of a chrome liquor in limited quantity, sufficient only to impart the characteristics of chrome tannage to the leather.

2. A method of combined tannage of hides and skins, to produce heat and moisture resistant leather, which comprises the successive treatment of the hide with solutions including a soluble pyrophosphate and including a chrome liquor, the latter being employed in proportions varying from one to eight per cent of the weight of the hide substance treated.

3. A method of combined tannage of hides and skins, to produce heat and moisture resistant leather, which comprises subjecting the hide to the tanning action of a solution of a soluble pyrophosphate and a soluble aluminum salt, and adding a chrome liquor to the solution during the tanning operation in proportions varying between one and eight per cent of the weight of the hide treated.

4. A method of combined tannage of hides and skins, to produce heat and moisture resistant leather, which comprises subjecting the hide to the tanning action of a solution of a soluble pyrophosphate and a soluble aluminum salt, and gradually adding a chrome liquor to the solution during the tanning operation in proportions varying between one and eight per cent of the weight of the hide treated.

In testimony whereof I affix my signature.

ERNEST WYNDHAM MERRY.